

No. 878,931.

PATENTED FEB. 11, 1908.

H. S. BERLINER.

METHOD OF MAKING GRAMOPHONE RECORD TABLETS.

APPLICATION FILED NOV. 11, 1907.



Witnesses

*C. E. Steff*  
*J. M. Maiford.*

Inventor

*Herbert S. Berliner.*  
By  
*Eugene C. Johnson*  
Attorney

# UNITED STATES PATENT OFFICE.

HERBERT S. BERLINER, OF WASHINGTON, DISTRICT OF COLUMBIA.

## METHOD OF MAKING GRAMOPHONE-RECORD TABLETS.

No. 878,931.

Specification of Letters Patent.

Patented Feb. 11, 1908.

Application filed November 11, 1907. Serial No. 401,725.

*To all whom it may concern:*

Be it known that I, HERBERT S. BERLINER, a citizen of the United States of America, residing at Washington, in the District of Columbia, have invented certain new and useful Improvements in Method of Making Gramophone-Record Tablets; and I do hereby declare the following to be a full, clear, and exact description of the invention, such as will enable others skilled in the art to which it appertains to make and use the same, reference being had to the accompanying drawings, which form a part of this specification.

15 This invention has reference to the manufacture of gramophone sound-record tablets, and has for its object to reduce the cost of production without impairing the durability or wearing qualities of the record.

20 In carrying my invention into effect, I first make a mixture of the ingredients or elements that ultimately form the surface in which the sound-grooves are impressed, and such mixture may be made up of barites, 25 silica or other earthy matter, a fiber, as cotton-flock, asbestos, shoddy or light fibrous material, with shellac, and when desired coloring matter may be added.

The above named ingredients or the 30 equivalents thereof are thoroughly incorporated or mixed together by heating and kneading, the mixture being rolled into sheets forming a solid mass when cool. This solidified base composed of granular material, a fiber, and shellac, is reduced by 35 grinding to a fine powder, and such grinding of the hard or solid mass which has a fiber intermixed therewith produces a fine powder in which the fiber is thoroughly incorporated.

40 It is important to note that, in order to grind the fiber into a powder, it must be incorporated into a hard cold mass forming a part thereof, and this is one of the particulars of my improvement over other methods which 45 enables me to subsequently produce an entirely homogeneous fibrous fluid for coating the hard base of my record.

Having reduced the fibrous mass to a fine powder, I next bring it to fluidity by the addition of alcohol, or other fluid solvent of shellac, the amount of alcohol or liquid that is added being sufficient to reduce the dry powder to a viscous fluid, and such fluid is applied either to one or both sides of a solid base 50 or foundation, for instance, a disk of pasteboard, wood, metal or resinous composition,

or to a sub-base, as a sheet of paper, which may then be reinforced by a backing, and when one coat or covering has been applied and has dried a second coat may be applied, 60 and so on until a surface of the desired thickness is secured. The coat or coatings may be applied by a brush or roller, and when the solvent has evaporated, the mixture solidifies and forms a hard coating. Before im- 65 pressing the sound-record into the surface of the tablet or disk it is heated to render the sound-record surface plastic, after which the sound-grooves are impressed therein in the usual manner, the disk being cooled while 70 under pressure and while in close contact with the sound-record matrix.

I desire to cover in this application the method described for producing an entirely homogeneous fibrous fluid for making a 75 gramophone record surface, and I do not broadly claim herein the general idea of coating a disk with a gramophone record composition in fluid form, drying the latter and impressing a record therein. 80

The method or process is illustrated by the accompanying diagram.

I claim:

1. The method of making gramophone sound-records, consisting in kneading the 85 materials which are to form the record surface, one of the materials being a fiber, the mixture being effected in the presence of heat, grinding the resulting mixture when cooled into a fine powder, mixing the powder 90 with a proper liquid for changing the same into a viscous fluid, applying one or more coats of such fluid to one or both sides of a disk, drying the surface, and impressing a sound-record into said surface-coated-disk 95 under heat and pressure.

2. The herein described method of making sound-record tablet surfaces for gramophones, which consists in kneading under heat the materials, including a fiber, which 100 ultimately form the record-surface, grinding the resultant mass after cooling to a fine powder, reducing the powder to a viscous fluid by mixing the same with a liquid, applying one or more coats of said fluid to a 105 base or sub-base, to form when dried and subsequently softened by heat a surface in which the sound-grooves are impressed.

3. The herein described method of making a sound-record surface for gramophone tablets consisting in incorporating by heating 110 and kneading an earthy base, shellac, and

fiber, to form when cool a solid mass, reducing such mass by grinding to a fine powder, mixing the powder with alcohol to form a viscous fluid, covering a base or sub-base 5 with the mixture and when dry softening the applied mixture by heat preparatory to impressing the sound-grooves therein.

4. The method for making a surface for sound-record tablets, which consists in 10 incorporating by kneading under heat an earthy granular base, fiber and shellac, with or without a pigment, cooling the same to form a solid mass, grinding the mass to a fine

powder, mixing such powder with a fluid to reduce the same to fluidity, applying such 15 mixture to a suitable base or sub-base to form when dried and subsequently softened by heat a surface in which the sound-grooves are impressed.

In testimony whereof I affix my signature 20 in presence of two witnesses.

HERBERT S. BERLINER.

Witnesses:

DAVID ROTHSCHILD,  
JOSEPHINE AMES.